

# United States Patent Office

2,931.714

Patented Apr. 5, 1960

1

2,931,714

# MOTOR GASOLINE CONTAINING BORON AND HEXYLENE GLYCOL

Richard J. de Gray, Shaker Heights, Ohio, assignor to The Standard Oil Company, Cleveland, Ohio, a corporation of Ohio

**No Drawing. Application November 4, 1957  
Serial No. 694,127**

**3 Claims. (Cl. 44—63)**

This invention relates to a motor gasoline containing small amounts of a boron compound from a class described hereinafter and hexylene glycol which demonstrates unexpected improvement in octane rating. It is intended that the motor gasoline of this invention also may include tetraethyl lead and other additives commonly employed in commercial gasolines today, such as oxidation inhibitors, gum inhibitors, dyes, solvents, and the like.

There has been an increasing demand, due to the recent trend of higher compression ratios in automotive engines, for gasolines exhibiting higher anti-knock qualities. This anti-knock characteristic of gasolines is commonly expressed in octane numbers wherein the fuel under consideration is compared to blends of standard compounds, i.e., iso-octane (2,2,4-trimethyl pentane) which is assigned an arbitrary number of 100, and n-heptane which is assigned an arbitrary number of 0.

In the race to develop such higher anti-knock qualities for motor gasoline, a difficult problem presents itself to the refiner, requiring skillful variations in refining operations and gasoline stock blending in order to obtain the anti-knock improvement required. This pressure on refining operations can be relieved measurably by chemical additives which in part can accomplish this increase in octane rating.

The octane number of gasoline is measured in laboratories by two independent tests referred to as the research method and the motor method. Both tests are performed in a single cylinder ASTM engine with the gasoline to be tested used as the fuel. A device is installed in the cylinder head of this ASTM engine so that the pressure impulses from detonation can be detected. These are electronically amplified and their intensity indicated on a knock meter on the engine panel board. The unknown fuel is compared in knock intensity with that of various reference fuels which are blends of the two standard compounds, iso-octane and n-heptane. A blend of iso-octane and n-heptane is found which produces the same knock intensity as does the unknown gasoline. The percentage by volume of iso-octane in the matching blend is designated as the octane number of the gasoline. For example, if a blend of 80% iso-octane and 20% n-heptane is required to duplicate the knock intensity of the unknown gasoline, the gasoline would then be given an octane number of 80.

Operating conditions for the engine vary depending upon whether a rating by the research method or the motor method is being determined. The operating conditions for this ASTM engine when running the research method determination is set forth in ASTM D 908-55. The operating conditions for this ASTM engine when running the motor method determination is set forth in ASTM D 357-53. In general, the motor method is a more severe test than the research method. Accordingly, most gasolines will have a higher octane number by the research method than by the motor method. It is felt that the

2

octane number determined by the research method correlates more closely with gasoline performances in engines running at low speed, whereas the octane number determined by the motor method is felt more indicative of gasoline performance under conditions of high speed and hence the octane number by this method is considered more significant as a measure of how the gasoline will perform in an automotive engine in actual road operation in today's automobiles with automatic transmissions which generally run at higher speeds.

It is therefore the object of this invention to offer a gasoline which contains small percentages of an additive combination which is effective in improving the octane rating of commercial gasolines, particularly when measured in accordance with the motor method.

In accordance with this invention, it has been found that hexylene glycol, when added to a gasoline containing a boron compound from a class which is known to produce beneficial effects by its incorporation into motor fuels, coacts with the boron compound to provide an unexpected improvement in octane rating.

Hexylene glycol as used herein is intended to mean a saturated aliphatic diol which is either a straight-chain compound or a straight-chain compound with one branch chain, non-limiting examples of which are hexane diol-2,5; 2-methyl pentanediol-2,4; and 2-ethyl butanediol-2,4. Of these examples, 2-methyl pentanediol-2,4 is preferred.

Of these examples, 2-methyl pentanedioi-2,4 is preferred. Patent No. 2,741,548, granted to my associates and assigned to my assignee, discloses a class of boron compounds which when incorporated into leaded gasolines and utilized in automotive engines are effective in suppressing surface ignition, increasing spark plug life, reducing total combustion chamber deposits, and other advantages. Included in the compounds described in this patent are those having the formula:



or the formula:



The former compound, which may be named 2-methyl pentanediol-2,4 hydrogen borate, will be referred to hereinafter as the boron ester; and the latter compound, which may be named bis-(2-methyl pentanediol-2,4) diborate, will be referred to hereinafter as the boron anhydride.

These compounds, separately or together in any proportions, are used in gasolines in the amounts of 0.025 to 0.1%, based on total fuel present. The presence of such amounts of these baron compounds in gasoline is found to exhibit a positive effect on the research method rating of the fuel and a significant negative effect on the motor method rating of the fuel.

It has been determined that the presence of hexylene glycol in gasoline not containing boron does not appreciably alter octane number by either the research method or the motor method. The addition of small concentrations of hexylene glycol in the range of from 0.03 to 0.1%, based on the total fuel present to a boron-containing gasoline does not diminish the octane number by the research method and demonstrates a surprising and

unexpected effect in increasing the motor method octane rating of the fuel.

A more complete understanding of the invention will be gained from the following results in which the base fuel common to all tests had an octane rating of 99+ and the following distillation characteristics:

|                     |      |      |    |  |  |
|---------------------|------|------|----|--|--|
| IBP                 | ° F. | 98   |    |  |  |
| 10%                 | ° F. | 128  |    |  |  |
| 20%                 | ° F. | 144  |    |  |  |
| 30%                 | ° F. | 162  | 10 |  |  |
| 40%                 | ° F. | 178  |    |  |  |
| 50%                 | ° F. | 201  |    |  |  |
| 60%                 | ° F. | 224  |    |  |  |
| 70%                 | ° F. | 256  |    |  |  |
| 80%                 | ° F. | 303  | 15 |  |  |
| 90%                 | ° F. | 362  |    |  |  |
| EP                  | ° F. | 424  |    |  |  |
| Reid vapor pressure |      | 8.75 |    |  |  |

| Fuel                                                     | F-1<br>O.N. | $\Delta$<br>Effect of<br>Hexylene<br>Glycol | F-2<br>O.N. | $\Delta$<br>Effect of<br>Hexylene<br>Glycol |
|----------------------------------------------------------|-------------|---------------------------------------------|-------------|---------------------------------------------|
| Base Fuel                                                | 99.7        |                                             | 90.9        |                                             |
| Base Fuel+Hexylene Glycol <sup>1</sup> (0.05%)           | 99.6        | -0.1                                        | 90.9        | 0.0                                         |
| Boron Fuel [Base Fuel+<br>Boron <sup>2</sup> (0.004% B)] | 99.9        |                                             | 90.1        |                                             |
| Boron Fuel+Hexylene Glycol <sup>1</sup> (0.05%)          | 99.9        | 0.0                                         | 90.7        | +0.6                                        |

<sup>1</sup> Hexylene glycol above refers to 2-methyl pentanediol-2,4.

<sup>2</sup> Boron above refers to a boron reaction mixture of which 75% of the mixture is boron anhydride and 25% of the mixture is boron ester, as previously described. The boron mixture is supplied to the gasoline in amounts to supply 0.004% by weight boron to the fuel.

As may be noted in the table above, the addition of hexylene glycol to the boron-containing fuel did not affect the research method octane number. The hexylene glycol addition, however, has a marked and surprising effect on the motor method octane number, increasing it 0.6 or more than one-half an octane number. At the high octane level of the boron-containing gasoline used in this test any further increase in octane number, especially by the motor method without any loss in the research method number, normally proves difficult and hence the surprising increase obtained by this slight addition of hexylene glycol is commercially significant.

The hexylene glycol in the amounts contemplated for this invention also serves as an excellent solvent for the boron compound in the invention, eliminating the need for an extra solvent which would otherwise be required in order to stabilize the boron composition in the liquid phase and lower its viscosity so the boron compound may be readily pumped and metered in the blending-in operation with gasoline. Hence, in the application of this invention the hexylene glycol may be added to the boron compound to provide the added ratio of these

two materials as desired in the final gasoline, and the mixture is then at a desired viscosity and adequately stabilized in the liquid phase for subsequent one-step blending into the gasoline.

I claim:

1. A motor gasoline to which has been added from 0.03 to 0.1% by weight hexylene glycol and 0.025 to 0.1% by weight of a boron compound having the formula:



where X is selected from the group consisting of hydrogen and



2. A motor gasoline to which has been added about 0.03 to 0.1% by weight hexylene glycol and an amount of a boron reaction mixture consisting of an admixture of about 25% the compound of the formula:



and 75% the compound of the formula:



to provide 0.004% by weight boron to the gasoline.

3. The gasoline of claim 2 in which the hexylene glycol is 2-methyl pentanediol-2,4.

#### References Cited in the file of this patent

#### UNITED STATES PATENTS

- |           |                |               |
|-----------|----------------|---------------|
| 2,315,957 | Hewlett        | Apr. 6, 1943  |
| 2,701,754 | Haworth et al. | Feb. 8, 1955  |
| 2,741,548 | Darling et al. | Apr. 10, 1956 |
| 2,767,069 | Fay et al.     | Oct. 16, 1956 |

UNITED STATES PATENT OFFICE  
CERTIFICATE OF CORRECTION

Patent No. 2,931,714

April 5, 1960

Richard J. DeGray

It is hereby certified that error appears in the above numbered patent requiring correction and that the said Letters Patent should read as corrected below.

In the grant, line 1, and in the heading to the printed specification, line 4, name of inventor, for "Richard J. de Gray", each occurrence, read -- Richard J. DeGray --; column 2, line 61, for "baron" read -- boron --.

Signed and sealed this 13th day of September 1960.

(SEAL)

Attest:

KARL H. AXLINE

Attesting Officer

ROBERT C. WATSON  
Commissioner of Patents